

Mar. 13, 1923.

1,448,084

T. F. OTT

METHOD OF PRODUCING LUBRICATING OILS

Filed May 1, 1920



INVENTOR.  
Thomas F. Ott  
BY  
Ackers & Follan  
his ATTORNEYS.

## UNITED STATES PATENT OFFICE.

THOMAS F. OTT, OF BERKELEY, CALIFORNIA.

## METHOD OF PRODUCING LUBRICATING OILS.

Application filed May 1, 1920. Serial No. 378,094.

*To all whom it may concern:*

Be it known that I, THOMAS F. Ott, a citizen of the United States, residing at Berkeley, in the county of Alameda and State of California, have invented certain new and useful Improvements in Methods of Producing Lubricating Oils, of which the following is a specification.

The invention resides in the treatment of the lubricating distillates or oils in such a manner as to produce in a single cycle of operation the light colored oils required or demanded by the public, and which it is the desire of the manufacturer to supply, but which heretofore has not been accomplished successfully except at a material increase in cost. The essential objects of the present invention are to produce light colored oils at a materially less expense than under the former methods employed; to expedite the manufacture of such colored oils; to successfully produce the desired light colored oils in a single cycle of operation and by so doing materially increasing the daily output of a plant of given capacity, and to dispense with the filtration of the oil through a filtering medium of "fuller's earth," and which filtering step is essential in such previous methods employed and generally followed in all manufacturing plants for the production of light colored oils.

Prior to the present invention the recognized and accepted standard method or process of treating lubricating distillates or oils for the production of light color oils, embodied essentially the following steps. First agitating the distillate or oil with sulphuric acid, settling out and withdrawing the sludge produced by the acid re-action; second, a subsequent agitation or spraying with a suitable neutralizing agent, for instance, sodium hydroxide, a settling out and withdrawal of the waste alkali and possible products of reaction; third, washing by agitation or spraying with water, until the oil is free of the alkali, and the settling and withdrawal of the waste water; and fourth, the heating of the oil and blowing air through the same until it is free or substantially free of all moisture. These steps followed in the order given constitute a single cycle operation, but the lubricating oil so produced was generally of a red color

and in order to produce the pale or light colored oils in popular demand by the public for gasoline motors, it was required to carry the method a step farther, viz: filter the oil so produced through a decolorizing agent, usually by passing the same through a tank or filter filled with fuller's earth.

Each manufacturer varied as desired the quantity of sulphuric acid used and neutralizing agent employed and equally so the time periods of treatment, but for a full understanding of said standard method, the following description is illustrative:

Approximately, seven hundred (700) barrels of lubricating distillate were placed in an acid agitator, a conical bottomed vessel having a holding capacity of about one thousand (1000) barrels. The oil was then agitated in the presence of about seventy-two hundred (7200) pounds of 98% sulphuric acid added thereto, by means of compressed air for a period of approximately thirty (30) minutes. After agitation settling was allowed for approximately two hours and the "sludge" formed drawn. The oil was then subjected to a second agitation with an additional ninety-seven hundred (9700) pounds of sulphuric acid for a period of about thirty minutes, settling allowed for sixteen hours and the sludge drawn off as before. Agitation was again resorted to and an additional thirty two hundred (3200) pounds of acid was added and, at the expiration of thirty minutes "blowing" with acid, water was sprayed over the surface of the oil. This water is known as "coking" water and its addition during agitation was to collect and agglomerate the very fine particles of "sludge" formed by the action of the acid on the oil, into particles of such size as to settle out fairly easily. No "coking" medium was required during the two first agitations, due to the fact that the first two increments of acid resulted in the formation of a sludge not so finely divided and which consequently settled out with ease. Following the application of the "coking" medium, settling was allowed for one hour, the sludge drawn off and the oil transferred from the acid agitator into an alkali agitator, similar in construction to the acid agitator. A hot solution of sodium hydroxide was sprayed onto the oil until about 160 barrels had been

100  
105

added and settling was then allowed for two hours. The waste alkali and possible reaction products were drawn off and fresh alkali added until the oil was thoroughly neutralized. The alkali was settled out as well as possible by standing about 16 hours and then drawn off. The oil was then washed by spraying on hot water to remove any traces of alkali and the water settled out as perfectly as possible and drawn off. However, mere settling not being sufficient to remove all traces of moisture, the oil was then transferred to a rather shallow, rectangular tank known as the "blow pan." In this blow-pan the oil was heated by means of closed steam coils and compressed air passed through it until the oil was perfectly bright and free from moisture.

The resulting oil was generally of a red color and in order to produce the pale or light colored oils in popular demand for gasoline motors, it was necessary to filter this oil through a tank filled with fuller's earth, which is a decolorizing agent.

This was a slow and expensive process and at various times it was endeavored to produce light colored oils by increasing the amount of acid in the chemical treatment. However, results were not encouraging, and, in fact, the larger amounts of acid used seemed to result in an even darker red oil in the blow-pans. Even when employing the larger amounts of acid, additions were always made in three increments, although the relative proportions of the increments were varied. One "coking water" was always used after the last increment of acid.

Efforts were made to get a light colored oil by using a larger amount of acid by taking the oil from the blow-pan and putting it back in the acid agitator and so subject it to a complete additional cycle of chemical treatment.

As the usual practice was to give a "treat" of oil about 20,000 pounds of acid, or practically thirty pounds of acid per barrel of oil, the oil when put through two cycles not only received double the amount of acid, but also of alkali and water. In the second cycle the sludge formed by the action of the acid was less in amount than during the first cycle, but of such a quantity, which combined with the additional losses suffered in the alkali agitator, served to make this method of obtaining pale oils an expensive one as well as a slow one. These losses, which may run as high as five per cent of the oil being treated with each alkali wash, added to the cost of the alkali and operating costs, make a two cycle treatment uncommercial, but I am enabled by my invention to produce a decolorized oil economically and in a shorter period of time.

In order to produce the pale or light colored oil by a single cycle treatment and

at the same time dispense with the use of fuller's earth filtration or other de-coloring agent after treatment of the oils in the alkali agitator, I discovered the following method of treatment, which will be readily understood by reference to the accompanying sheet of drawings wherein is represented diagrammatically the movement of the oil through a single cycle treatment.

The usual amount of oil, about seven hundred barrels, is placed within the agitator 1 and during agitation subjected to the action of forty thousand pounds of sulphuric acid, the acid being added in four or five increments. After the first increment of say, eight thousand pounds, the oil is agitated for fifteen minutes, and settling allowed for two hours. The sludge is then drawn off through the controlled outlet 2 of the agitator 1, and a second increment of eight thousand pounds of acid added to the oil and the same agitated for fifteen minutes, and allowed to settle for approximately sixteen hours before drawing off the sludge. The oil is then subjected to a third agitation with eight thousand pounds of acid for a period of fifteen minutes and during agitation treated with about seven barrels of coking water for agglomerating and collecting the small particles of sludge contained therein and allowed to settle for six hours. The oil is then subjected to two additional agitations, with each there being added eight thousand pounds of acid, the agitation and settling being as before, coking water or other coking agent being sprayed onto the oil during each period of agitation after the adding of the acid. It will be understood that after each settling period the sludge formed by the acid reactions is drawn off, although the settling between increments of acid is a variable factor, dependent on the character of oil to be treated. After subjecting the oil to the last of the series of applications of coking water and the withdrawal of the sludge, the oil then freed of the sludge formed by the re-actions of the sulphuric acid is transferred to an alkali agitator 3, similar in all respects to the agitator 1 and, as common in the art of treating the oil sprayed with a hot solution of sodium hydroxide until about one hundred and sixty barrels are added and the oil then allowed to settle for about two hours. The waste alkali is drawn off and fresh alkali added until the oil is thoroughly neutralized. From this point on and in fact from the time of transference of the oil into the alkali agitator, the method is the same as that heretofore followed, except that after treatment in the acid agitator the oil is not passed through fuller's earth or subjected in any manner to decolorizing agents, such being rendered unnecessary by reason of the fact that subjecting the oil to

a plurality of coking treatments while contained within the acid agitator dispenses with filtration by the removal from within the oil of the sludge formed by the reactions 5 of the sulphuric acid.

The several coking treatments or "multiple-coking" employed or utilized in my process permits of an increased amount of sulphuric acid being utilized in one cycle of 10 operation. While the use of water as a coking medium is specifically mentioned in the treatment of the oils, it will be understood that water is not essential as the coking medium, inasmuch as a weak solution of sodium hydroxide and a weak acid solution 15 have been utilized by me with success, provided that the solution of sodium hydroxide is dilute enough to have no appreciable neutralizing effect upon the mixture of oil and acid, and, therefore, by the expression coking medium or coking agents as hereinafter employed, is meant to be understood the utilization of water or any other permissible solution as the coking medium, but preferably 20 I use water inasmuch as the use of weak sodium hydroxide or weak acid adds materially to the cost of the process without producing other beneficial result by their use in the place of water.

25 The use of the multiple coking employed in the step for eliminating the reaction products of the sulphuric acid is the simplest, cheapest and easiest way for most completely removing the sludge formed in the acid agitator after each increment of acid.

30 It is essential that multiple coking be utilized in order that the reaction products of the acid employed in connection with one treatment be removed as completely as possible before adding fresh acid, for, otherwise, the increased amount of sulphuric acid tends to oxidize or "burn" the oil.

35 While the maximum amount of acid used in the carrying out of my method is generally double that used in the former methods employed for the treatment of the oils, or roughly sixty pounds of acid per barrel of oil treated, yet the amount of acid is adjusted according to the degree of color desired in the finished product, and experience has demonstrated that quite a few of the oils do not require double the amount of acid to be utilized in my single cycle operation, over the quantity of acid employed in the carrying out of the former methods.

40 While the number and size of the increments of acid employed is not fixed, practical experiments have demonstrated that preferably these should be five in number, and while the coking treatment may be a variable one, the same should never be less than two in number.

45 Contrary to popular conception, the use of the additional amount of sulphuric acid required in the carrying out of my process

does not result in a smaller yield of the finished lubricating oil, for the percentage losses in this process are no higher than in the former methods employed.

The invention desired to be protected 70 resides in subjecting the distillates or oils for treatment to a plurality of agitating periods, each period being followed by a period of settlement and each period of agitation being in the presence of a fixed quantity of 75 sulphuric acid added to the oil and subjecting the oil during certain successive agitating treatment to the application of a coking medium, the coking medium being applied to the oil during the successive agitating periods thereof, and in number the coking treatments of the oil being never less than two, whereby the oil is freed of the sludge formed by the acid reactions, so that when delivered from within the alkali agitator the 80 same is of the light color desired.

85 It will be understood that the foregoing description does not necessarily represent, and is not intended to represent, the exact treatment for all oils under the present 90 method invention, inasmuch as the quantity of acid coking material, and the quantity and number of acid increments should be varied in accordance with the character of the oil to be treated or to be obtained.

95 Having thus described my invention, what I claim as new and desire to protect by Letters Patent is:—

1. The method of treating oils for the production of light colored lubricating oils 100 without subjecting the same to the action of a decolorizing agent after the acid treatment thereof, the same consisting in subjecting the oil to successive periods of agitation and settlement, adding a given quantity of 105 sulphuric acid to the oil during each period of agitation, and during a plurality of said successive agitations subjecting the oil to the action of water for the collecting and separation of the sludge formed by the acid 110 reactions, thence subjecting the oil freed of the sludge to a treatment with an alkali solution.

2. The process of decolorizing oils which 115 consists in mixing acid with an oil by a number of increments, adding water to each oil and acid mixture after more than one of the acid increments, removing acid sludge after each acid increment, then washing with an alkali after removal of the acid sludge resulting from the final acid increment.

3. The process of decolorizing oils which 120 consists in mixing acid with an oil by a number of increments, adding water to each oil and acid mixture after the first two increments, removing acid sludge after each acid increment, then washing with an alkali after removal of the acid sludge resulting from the final acid increment.

4. The process of decolorizing oils which 125

consists in mixing acid with an oil by five increments, adding water to each acid mixture after more than one of the acid increments, removing acid sludge after each acid increment, then washing with an alkali after removal of the acid sludge resulting from the final acid increment.

5. The process of decolorizing oils which consists in mixing acid with an oil by a number of increments, adding water to each oil and acid mixture after more than one of the acid increments, removing acid sludge after each acid increment, then washing with an alkali after removal of the acid sludge resulting from the final acid treatment; the number of acid increments being not less

than five and the number of water additions being not less than two.

6. The process of decolorizing oils which consists in agitating a lubricating oil with sulphuric acid, which acid is added in successive increments, mixing water with the oil and acid mixture during the third and succeeding acid increments, removing acid sludge after each increment, then washing with an alkali after removal of the acid sludge resulting from the final acid increment, and drawing off alkali waste liquors.

In testimony whereof I have signed my name to this specification.

THOMAS F. OTT.